# EUROPEAN PATENT SPECIFICATION

(11) **EP 0 272 687 B1**
(45) Date of publication and mention of the grant of the patent: **28.06.1995**
(21) Application number: 87119051.8
(22) Date of filing: 22.12.1987
(51) Int. Cl.: H01J 61/073, H01J 61/067, H01K 1/08

(54) **Tungsten duplex composite electrode and filament material**
Elektrode und Drahtmaterial aus Wolfram von zweifältiger Zusammensetzung
Matériau pour une électrode ou un filament composé en tungstène

(30) Priority: 22.12.1986 US 945746
(43) Date of publication of application: 29.06.1988
(73) Proprietor: GTE PRODUCTS CORPORATION, Wilmington Delaware 19801 (US)
(72) Inventor: Passmore, Edmund M., Gloucester, MA 01930 (US); Patrician, Thomas J., Monroeton, PA 18832 (US)
(74) Representative: Grünecker, Kinkeldey, Stockmair & Schwanhäusser Anwaltssozietät

(56) References cited:
- EP-A- 0 019 992
- DE-A- 3 036 746
- FR-A- 1 234 443
- FR-A- 1 464 066
- GB-A- 2 079 531
- PATENT ABSTRACTS OF JAPAN vol. 5, no. 59 (E-53) 22 April 1981 ; & JP-A-56 118 32
- PATENT ABSTRACTS OF JAPAN vol. 2, no. 64 (E-33) 17 May 1978 ; & JP-A-53 30 266
- PATENT ABSTRACTS OF JAPAN vol. 8, no. 258 (M-340) 27 November 1984 ; & JP-A-59 130 697
- PATENT ABSTRACTS OF JAPAN vol. 6, no. 91 (E-109)(969) 28 May 1982 ; & JP-A-57 256 64
- LAMPS AND LIGHTING, S.T. Henderson and A.M. Marsden, Thorn Lighting Ltd., 1972, pp. 142-147.

## Description

### BACKGROUND OF THE INVENTION

The present invention is directed to a duplex composite member suitable for use in lamps, as either an electrode and/or a filament element. This duplex composite member has two component parts; (1) a core composed of one type of tungsten-based material, and (2) a shell composed of a different tungsten-based material.

The duplex composite member of the present invention may have desirable surface properties such as resistance to chemical attack and/or mechanical shock and vibration, making it especially well suited for applications in incandescent lamps, metal halide discharge lamps, and/or halogen incandescent lamps.

Electrode and/or filament failure due to mechanical shock and/or chemical attack is a recognized problem in the lighting industry. For example, U.S. Patent No. 4,413,205 describes in detail how the tungsten conductors to the coiled filament of a halogen incandescent lamp are locally pitted and chemically attacked by bromine in such a manner that they break and the lamp fails.

The US-A-4,413,205 patent suggests one method for reducing this chemical attack problem, namely, modifying the conductor material to a tungsten -rhenium (Re) alloy containing at least 0.1% Re.

Similarly, it is known that filament and/or electrode failure due to chemical attack can also occur in metal halide high intensity discharge (HID) lamps, especially where reactive halogens, including bromine, chlorine, and iodine have been used. See, for example J. F. Waymouth, "Electric Discharge Lamps" pg. 210, (1971).

The chemical attack of thoriated tungsten electrode rods thus constitutes a recognized obstacle in the application of the reactive halogens in metal halide discharge lamps.

Although such changes in electrode composition as those described in the US-A-4,413,205 patent may overcome the problem of electrode failure due to chemical attack, such alloys suffer from two major shortcomings:
(a) they do not possess the necessary emissive characteristics of the W - (usually 1 - 2%) Th0₂ materials typically used for electrodes and
(b) they introduce excessive Re emission into the light emitting plasma discharge of metal halide lamps.

From JP-A- 56-11832 there is known a directly heated cathode of a electron tube constituting of a tungsten core wire having a coating layer of sodium carbide or a tungsten carbide-thorium alloy formed on its outer surface.

DE-A-30 36 746 discloses an arc lamp having an anode made of tungsten with Si, Al and/or K as dopants.

Finally, from the publication "Lamps and Lighting", Henderson & Marsden, 1979, page 144 it is known to fabricate tungsten wires from sintered bars containing dopants.

The present invention is directed to an alternate solution to the problems of chemical attack and/or mechanical shock of electrodes and/or filaments, which does not suffer the disadvantages discussed above.

### SUMMARY OF THE INVENTION

The present invention provides a method of fabricating a composite lamp member in accordance with claim 1.

The dependent claims describe particular embodiments of the invention.

One example of the benefits which may be conferred by the present invention is exemplified by the manner in which the aforementioned difficulties of the prior art may be avoided. In one embodiment of the present invention, an electrode is formed from a duplex composite member, composed of a thoriated tungsten core (W - Th0₂) and a thin tungsten-rhenium (Re) shell. In this embodiment, any rhenium emission is limited to an insignificant amount (i.e., that vaporized from the thin shell, especially at the tip of the electrode).

Other embodiments of duplex composite members are provided by thoriated tungsten discharge electrodes in which it is desirable to have two different concentrations of thoria (ThO₂) in the element, a first concentration in the core of the duplex composite member and a second concentration in the shell or surface of the member. In preferred embodiments, the thoria concentration in the shell portion of the duplex composite may be either lower or high than the thoria concentration in the core portion.

One desirable objective which can be facilitated by the use of the duplex composite member of the present invention is the ability to draw thoriated core tungsten to much finer sizes (i.e., smaller diameters) than heretofore feasible.

Prior to the present invention, the limit of wire sizes for thoriated tungsten (with much greater than about 1% ThO₂) was no lower than about 0,51 mm (0.020 inch) in diameter. By utilizing a duplex composite member of the present invention composed of a 2% thoriated tungsten cure with a 1% thoriated tungsten shell, drawn wire of 0,43 mm (0.017 inches) in diameter has readily been prepared. Unlike the 0,51 mm (0.020 inch) diameter wire previously prepared, this 0,43 mm (0.017 inch) diameter wire is especially well suited for use in low wattage metal halide lamps, i.e. 40 to 100 watts.

### DETAILED DESCRIPTION OF THE PREFERRED EMBODIMENTS

As set forth above, the present invention provides a tungsten-based duplex composite member, e.g., wire or rod, which combines the emissive, nonsag, or other desirable qualities of an inner tungsten-based core material, with a different combination of properties, for example, resistance to attack, by the presence of a different tungsten-based material as an outer sheath or shell surrounding the core material.

As used herein, the term "tungsten-based material" is defined as tungsten-containing compositions suitable for use as filament and/or electrode members in lamps, especially incandescent lamps, metal halide discharge lamps, and halogen incandescent lamps. Typically tungsten makes up at least about 95 percent (by weight), or more, of such compositions. After careful consideration of the teachings of the present disclosure, the skilled artisan will readily recognize suitable compositions for use herein.

Core materials may include thoriated tungstens, for example, tungsten compositions containing thoria in the range of from about 0.5 to about 5.0 percent (by weight). Other types of tungsten-based materials which may constitute the core include nondoped, i.e., commercially pure (CP) tungsten, potassium (K) doped nonsag tungsten (normally used in incandescent filaments), and tungsten alloys. Such materials are known to the skilled artisan in the lighting field.

Other core materials include tungsten modified with emissive materials such as CeO₂, La₂O₃, Sc₂O₃, HfO₂, ZrO₂, and the like, in concentrations ranging up to about 5 percent (by weight). Combinations of these emitters with and without thoria may also be employed as a tungsten-based core material herein.

Another example of a useful tungsten-based core material is provided by Japanese Patent No. 58-129741 which describes the use of a tungsten electrode containing 20 ppm aluminum (Al). This Al level substantially exceeds currently specified levels of this element in wire).

As shell materials, any of the above described core materials may be employed, with the proviso that the core material and the shell material of any given duplex composite member are not the same.

In addition, attack and corrosion-resistant tungsten-rhenium alloys may also be used as shell materials. Such (Re)alloys, containing up to about 5% Re (by weight) will also promote mechanical shock and vibration resistance, making the duplex composite member especially well suited for use as incandescent filaments for applications involving such shock and vibration, while minimizing the amount of expensive Re which must be used and enhancing the luminous efficacy by the use of a K-doped, nonsag core.

Such a combination with a tungsten-rhenium (W-Re) shell around a potassium (K)-doped, nonsag core enables the composite to be used as the filament of a halogen incandescent amp, in which separate internal conductors are not required.

In general, duplex composites are prepared by isostatically cold pressing the preblended and preplaced powders together into a billet with the core preplaced concentrically within the shell. The billet is then densified by sintering at a high temperature and reduced to wire of the desired diameters by the usual tungsten processing methods of rolling, swaging, and drawing.

The present invention will be further illustrated with reference to the following examples which will aid in the understanding of the present invention, but which are not to be construed as limitations thereof. All percentages reported herein, unless otherwise specified, are percent by weight. All temperatures are expressed in degrees Celsius.

### EXAMPLE I

Duplex composite electrodes with a 2% thoria core inside a 1% thoria shell were prepared for testing in both 100 watt and 400 watt metal halide lamps (Sylvania Metalarc lamps).

When viewed as a polished cross-section, the 2% thoria core is clearly revealed in contrast to the 1% thoria shell, which has a much coarser grain structure, being attributed to the larger grain size following the previous recrystallization-anneal.

The mold used in this example consisted of three main sections, a cylindrically shaped outer PVC mold support tube (156,25 mm I.D. x 500 mm) (2.25 in. I.D. x 20 in.); a cylindrically shaped outer mold member (50 mm I.D. x 1200 mm) (2 in. I.D. x 24 in.) and a cylindrically shaped stainless steel inner mold/fill tube (25 mm x 900 mm) (1 in. x 36 in.).

A portion of the upper section of the stainless steel inner mold/fill tube was flared out to a diameter of 50 mm (2 in.) to act as a funnel for the introduction of powders. At the bottom of the outer PVC mold support tube was placed a segment of hard rubber, which acted as a shock absorber.
The three component parts were concentrically fitted together and filling was conducted as described below.

The procedure used to prepare this duplex composite started by adding 3,000 grams of W-2% ThO₂ powder to the central fill tube of the mold described above. At the same time, 1,000 grams of W-1% ThO₂ powder was placed in the space between the mold and the central fill tube.

The entire assembly was gently tapped during the filling operation until the prescribed amounts of both powders were added to the mold. At the end of the filling operation the levels of powder in the core and the outer shell were approximately the same. One critical aspect of filling is that the powders are only loosely packed into the mold since tight packing prevents the removal of the central filling tube.

After filling and the extraction of the fill tube, the mold was sealed, then cold isostatically pressed at a pressure of approximately 310 MPa (45,000 lbs) per square inch. The pressed powder compact was then solid state sintered for about 12 hours at about 2,100°C in a hydrogen atmosphere producing a composite ingot weighing about 13 kg with a density of 17.6 g/cc, i.e., about 93% of the theoretical density.

The resulting ingot was about 1.5 inches in diameter by about 475 mm (19 inches) long. The W-1% ThO₂ shell comprised about 70% of the ingot volume with the W-2% ThO₂ making up the remainder, producing an ingot with an average ThO₂ content of 1.34% by analysis.

Reduction of the ingot began first by rolling on a two-high rolling mill from 37,5-25,0 mm (1.5 to 1.0 inch) in diameter in multiple-passes at a temperature above 1300°C. After recrystallization, the ingot was rolled twice at a temperature above 1400°C on a multiple stand rolling mill manufactured by Frederick Kocks Co., to a diameter of about 7,5 mm (0.3 inch) with an intermediate recrystallization.

The ingot was further reduced to about 0.1 inch diameter by multiple-pass swaging with three more recrystallization anneals. Because the diffusivity of ThO₂ in tungsten is very low for all of the processing temperatures employed herein, the interface between the W-1% ThO₂ outer shell and the W-2% ThO₂ core remains distinct, maintaining the duplex composite structure. Below 2,5 mm (0.1 inch) diameter the ingot was drawn into wire using conventional wiredrawing practices for W-ThO₂ wire.

The duplex composite wire made thereby was drawn to 0.039 inch diameter. Cathode rods for 400 watt metal halide lamps were prepared therefrom by centerless grinding to 0,91 mm (0.0365 inch) diameter and sectioning the ground rods into 1/2 inch lengths. These members were used to prepare seventeen 400 watt Metalarc-type lamps (having an arc tube fill comprising Na, Sc, I, and Hg) each of which lighted and operated normally in accordance with their design ratings.

The remainder of the 0,99 mm (0.039 inch) wire was drawn further to a diameter of 0,42 mm (0.017 inch) and this drawn wire was sectioned into 0,73 mm (0.0295 inch) segments. These small segments were used to prepare five 100 watt metal halide lamps, also having an arc tube fill comprising Na, Sc, I, and Hg. These lamps operated normally after burning for over 2000 hours. They were also found to start slightly faster than the standard lamps having a 1% thoria cathode, in this case 91 seconds versus 95 seconds.

### EXAMPLE II

A duplex composite member is also prepared, using essentially the same procedures set forth in Example I, but with a non-thoriated core of tungsten encased in a shell of 2% thoria. 100 Watt Metalarc type amps made therefrom are found to start much faster than the standard Metalarc amps having a 1% thoria electrode. The lamps will also demonstrate improved lumen maintenance, especially when compared to prior art lamps with the same rapid starting characteristics, but wherein 2% thoriated tungsten makes up the entire electrode.

The present invention has been described in detail, including the preferred embodiments thereof. However, it will be appreciated that those skilled in the art, upon consideration of the present disclosure, may make modifications and/or improvements on this invention and still be within the scope of the following claims.

## Claims

1. A method of fabricating a composite lamp electrode and/or filament member, said member including a core formed from a first compacted tungsten-based material and a shell intimately bonded to the outer surface of said core, said shell being formed from a second compacted tungsten-based material, said method comprising the following steps:
(a) inserting said first tungsten-based material within a centered fill tube of a cylindrical mold;
(b) inserting said second tungsten-based material in powder form into the space surrounding said fill tube and within said mold;
(c) extracting said fill tube from said mold such that a composite cylindrical billet is formed within said mold;
(d) removing said billet from said mold;
(e) cold pressing said billet isostatically;
(f) sintering said billet thereby forming a composite ingot; and
(g) rolling, swaging, and drawing said composite ingot thereby forming a composite wire; and
(h) forming said composite lamp member from said wire.

2. A method of fabricating a composite lamp member as described in claim 1, wherein said shell includes a material selected from the group consisting of thoria in a concentration of 0,5 to about 5,0 percent and rhenium in an amount of 5 percent or less by wight.

3. A method of fabricating a composite lamp member as described in claim 2, wherein said core consists essentially of tungsten.

4. A method of fabricating a composite lamp member as described in claim 1, wherein said core and said shell both include the same material selected from the group consisting of thoria and rhenium in different amounts.

5. A method of fabricating a composite lamp member as described in claim 1, wherein said cold isostatic pressing of said composite billet is performed at approximately 310 MPa.

6. A method of fabricating a composite lamp member as described in claim 1, wherein said sintering of said billet lasts approximately twelve hours at approximately 2,100 degrees Celsius.

7. A method of fabricating a composite lamp member as described in claim 1, wherein said composite ingot has a density of approximately 93 percent of its theoretical density.

8. A method of fabricating a composite lamp member as described in claim 1, wherein said composite wire has a cross-sectional diameter of approximately 0,99 mm (0,039 inch).

9. A method of fabricating a composite lamp member as described in claim 1, wherein said composite wire has a cross-sectional diameter of approximately 0,43 mm (0,017 inch).

## Patentansprüche

1. Verfahren zur Herstellung eines Elektroden- und/oder Glühdraht (Filament)- Verbundelements für eine Lampe, wobei das Element umfaßt: einen Kern gebildet aus einem ersten verdichteten Material auf Wolframbasis und einem Mantel bzw. einer Hülle (Shell), die innige mit der Außenfläche des Kern verbunden ist, wobei die Hülle aus einem zweiten verdichteten Material auf Wolframbasis gebildet ist, das Verfahren umfaßt die folgenden Schritte:
a) Einführen des ersten Materials auf Wolframbasis in das Innere eines in einer zylindrischen Form zentrierten Füllrohres;
b) Einführen des zweiten Material auf Wolframbasis in Pulverform in den Raum, welcher das Füllrohr umgibt und in das Innere der Form;
c) Herausziehen des Füllrohres aus der Form, so daß ein zylindrischer Verbundbarren im Inneren der Form gebildet wird;
d) Entfernen des Barrens aus der Form;
e) Isostatisches Kaltpressen des Barrens;
f) Sintern des Barrens, wodurch ein Verbundblock gebildet wird; und
g) Walzen, Kalthämmern und Ziehen des Verbundblockes, wodurch ein Verbunddraht gebildet wird; und
h) Bilden eines Verbundelementes für eine Lampe aus dem Draht.

2. Verfahren zur Herstellung eines Verbundelements für eine Lampe nach Anspruch 1, worin die Hülle ein Material umfaßt, gewählt aus der Gruppe, bestehend aus Thoria in einer Konzentration von 0,5 bis ungefähr 5,0% und Rhenium in einer Menge von 5% oder weniger, bezogen auf das Gewicht.

3. Verfahren zur Herstellung eines Verbundelements für eine Lampe nach Anspruch 2, worin der Kern im wesentlichen aus Wolram besteht.

4. Verfahren zur Herstellung eines Verbundelementes für eine Lampe nach Anspruch 1, worin sowohl der Kern als auch die Hülle das gleiche Material umfassen, gewählt aus der Gruppe bestehend aus Thoria und Rhenium in unterschiedlichen Mengen.

5. Verfahren zur Herstellung eines Verbundelements für eine Lampe nach Anspruch 1, worin das isostatische Kaltpressen des Verbundbarrens bei ungefähr 310 MPa durchgeführt wird.

6. Verfahren zur Herstellung eines Verbundelements für eine Lampe nach Anspruch 1, worin das Sintern des Barrens wenigstens 12 Stunden bei ungefähr 2100° C andauert.

7. Verfahren zur Herstellung eines Verbundelements für eine Lampe nach Anspruch 1, worin der Verbundblock eine Dichte von ungefähr 93% seiner theoretischen Dichte aufweist.

8. Verfahren zur Herstellung eines Verbundelements für eine Lampe nach Anspruch 1, worin der Verbunddraht einen Durchmesser (Cross-sectional diameter) von ungefähr 0,99 mm (0,039 inch) aufweist.

9. Verfahren zur Herstellung eines Verbundelements für eine Lampe nach Anspruch 1, worin der Verbunddraht einen Durchmesser von ungefähr 0,43 mm (0,017 inch) aufweist.

## Revendications

1. Procédé de fabrication d'un élément composite d'électrode et/ou de filament pour lampe, le dit élément incluant un noyau formé à partir d'un premier matériau compacté à base de tungstène et une coquille intimement lié à la surface extérieure du dit noyau, la dite coquille étant formée à partir d'un deuxième matériau compacté à base de tungstène, le dit procédé comprenant les étapes suivantes :
(a) introduire le dit premier matériau à base de tungstène à l'intérieur d'un tube de remplissage centré d'un moule cylindrique ;
(b) introduire le dit deuxième matériau à base de tungstène sous forme d'une poudre dans l'espace entourant le dit tube de remplissage et à l'intérieur du dit moule ;
(c) enlever le dit tube de remplissage du dit moule, de telle manière qu'une billette cylindrique composite soit formée à l'intérieur du dit moule ;
(d) ôter la dite billette du dit moule ;
(e) presser à froid la dite billette de façon isostatique ;
(f) fritter la dite billette de manière à former un lingot composite ; et
(g) laminer, emboutir et étirer le dit lingot composite de manière à former un fil composite ; et
(h) former le dit élément composite pour lampe à partir du dit fil.

2. Procédé de fabrication d'un élément composite pour lampe selon la revendication 1 dans lequel la dite coquille comprend un matériau choisi dans le groupe comprenant de la thorine dans une concentration comprise entre 0,5 et 5,0 % environ et du rhénium en quantité inférieure ou égale à 5 % en poids.

3. Procédé de fabrication d'un élément composite pour lampe selon la revendication 2 dans lequel le dit noyau comprend essentiellement du tungstène.

4. Procédé de fabrication d'un élément composite pour lampe selon la revendication 1 dans lequel le dit noyau et la dite coquille comprennent tout deux le même matériau choisi dans le groupe comprenant la thorine et le rhénium en quantités différentes.

5. Procédé de fabrication d'un élément composite pour lampe selon la revendication 1 dans lequel le dit pressage isostatique à froid de la dite billette composite est réalisée sous approximativement 310 MPa.

6. Procédé de fabrication d'un élément composite pour lampe selon la revendication 1 dans lequel le dit frittage de la dite billette dure environ douze heures et est effectuée à approximativement 2100 degrés Celcius.

7. Procédé de fabrication d'un élément composite pour lampe selon la revendication 1 dans lequel le dit lingot composite présente une densité de 93 % environ de sa densité théorique.

8. Procédé de fabrication d'un élément composite pour lampe selon la revendication 1 dans lequel le dit fil composite présente un diamètre en coupe de 0,99 mm approximativement (0,039 pouce).

9. Procédé de fabrication d'un élément composite pour lampe selon la revendication 1 dans lequel le dit fil composite présente un diamètre en coupe de 0,43 mm approximativement (0,017 pouce).
